

A. & M. HIRSCH.

PROCESS OF MAKING CASTINGS OF RARE EARTH METALS AND THEIR ALLOYS.

APPLICATION FILED SEPT. 17, 1917. RENEWED NOV. 29, 1918.

1,290,011.

Patented Dec. 31, 1918.



Fig. 1.



Fig. 2.



Fig. 3.



Fig. 4.



Fig. 5.



Fig. 6.

INVENTORS  
Alcan Hirsch  
Mary Hirsch  
BY  
Gorham Crosby  
ATTORNEY

# UNITED STATES PATENT OFFICE.

ALCAN HIRSCH AND MARX HIRSCH, OF NEW YORK, N. Y., ASSIGNEES TO ALPHA PRODUCTS COMPANY, INC., A CORPORATION OF NEW YORK.

## PROCESS OF MAKING CASTINGS OF RARE-EARTH METALS AND THEIR ALLOYS.

1,290,011.

Specification of Letters Patent.

Patented Dec. 31, 1918.

Application filed September 17, 1917, Serial No. 191,663. Renewed November 29, 1918. Serial No. 284,718.

To all whom it may concern:

Be it known that we, ALCAN HIRSCH and MARX HIRSCH, citizens of the United States, and residents of New York, in the county 5 of New York and State of New York, have invented certain new and useful Improvements in Processes of Making Castings of Rare-Earth Metals and Their Alloys, of which the following is a specification.

10 The invention relates to improvements in the manufacture of castings of rare earth metals and their alloys and especially to the preparation of the metals for casting. The improvements are particularly adapted to 15 the manufacture of castings of alloys of cerium or lanthanum for sparking purposes.

Prior to the present invention it has been considered extremely difficult to cast the desired rods and shapes of cerium and its alloys 20 because of the extreme inflammability of the metal on the one hand and its great tendency to chemical reaction with carbon and other substances and to alloying with metals on the other hand. It was only by 25 the laborious and wasteful process of sawing or turning beneath the surface of oil, or while constantly drenching the fresh surfaces and cuttings with oil, that it was generally known how to make the small commercial 30 shapes necessary for use in lighters, ignition flints, etc.

The present process has for its object the providing of improvements whereby the rare earth metals and their alloys may be 35 satisfactorily cast in the various forms desired in commerce and, in many cases, with sufficient exactitude of size to avoid the necessity of machining, thereby avoiding not only delay and expense, but much loss of 40 material, which, once powdered, is extremely difficult to recover in usable shape. Also, according to the present invention, the cast metal or alloy is obtained in a most simple and economical manner and substantially 45 free from objectionable impurities.

Further and more specific objects, features and advantages will more clearly appear from the detailed description given below, taken in connection with the accompanying sheet of drawings, which forms a part of this specification.

In the drawing,

Figure 1 is a vertical section of a preferred form of apparatus for melting the 55 metals;

Fig. 2 is a top view of a mold into which the molten metal may be poured for casting;

Fig. 3 is a vertical section taken on the line 3—3 of Fig. 2;

Fig. 4 is a vertical section taken on the line 4—4 of Fig. 2;

Fig. 5 is a top plan view illustrating a modified form of mold; and

Fig. 6 is a similar view illustrating still another form of mold.

As an illustrative example of the improvements, the preferred process for the manufacture of castings of an alloy of cerium, lanthanum, didymium, etc., and iron will be described.

Large pigs of an alloy of cerium, lanthanum and didymium, and possibly small quantities of erbium and thorium, etc., and containing more or less impurities, are broken up, as with a hammer, into pieces 75 about one inch in diameter. It is preferred to avoid using much smaller pieces than one-half inch in diameter, as they tend to thicken the melt into which they are later put, probably because of the greater amount 80 of oxid formed on the surfaces of the pieces when an equal weight of smaller pieces is used. Larger pieces may be used, especially in the larger melts.

Into a suitable crucible, preferably a Hessian crucible, and suitably heated, a quantity of barium chlorid crystals is put and melted down. For this purpose, an apparatus such as shown in Fig. 1 may be used, in which 1 represents the crucible, 2 a supporting bed portion of firebrick, provided with gas flame blasts at 3, 3, directed against the bottom part of the crucible for heating the same. 4 represents a heat insulating jacket surrounding the crucible and 5 a heat insulating cover for the crucible, and 9 a cover surrounding the top of the crucible and resting on the jacket 4. Other forms of apparatus may, however, be used.

After the barium chlorid has been fused 100 in the crucible and the water contained in the barium chlorid crystals has been evolved and the mass reached a quiet state of fusion, the pieces of metal, consisting mostly of cerium with some lanthanum and small 105 quantities of other metals, are washed in kerosene or other suitable oil to remove dirt, oxids and carbids that may be on the surface thereof, and then they are partially dried, as with news print paper, and then 110

the pieces of metal are added to the melt of barium chlorid in fairly large batches, that is to say, as many pieces are added at a time as can be readily shoved under the surface of the barium chlorid. Any kerosene or other oil remaining on the pieces burns off as they go into the molten barium chlorid. The mass should not be stirred, and in adding the metal the melt should be agitated as little as possible. The cerium metal or alloy added should preferably be low in iron, as metal high in iron not only has a higher melting point, but is apt to contain more of other impurities and these impurities are then far more difficult to separate. We, therefore, prefer to use a rare earth metal containing about 10% or less of iron. When the metal added has become fluid at the bottom of the crucible, another batch of metal may be added in the same way and the molten metal batch built up, care being taken not to expose the already molten cerium metal in the melt to the air, which would rapidly ignite or oxidize it. The heating of the pieces of metal to melt them should be carried out relatively quickly, because, if the operation is carried out slowly, the metal melt does not become as clear and homogeneous, the fused salt above it becomes more viscous and difficult to separate from the metal, and much metal is apt to be lost, nor does the metal pour so well when it is later poured from the crucible. By relatively quickly, we mean that the whole operation of melting, alloying and casting the metal should take not over about two hours, instead of several hours.

When the crucible is about one-half full of molten metal, as illustrated at 6 in Fig. 1, any other metal which it is desired to alloy with it is added. In most cases, it is desirable to add certain other metals, such as iron, to harden the resulting alloy. This is added in the form of soft wrought iron wire. It is first cut off in pieces weighing, say, 40 to 50 grams and the pieces wound into loose coils or spools. These coils of wire are poked into the melt under the layer 7 of barium chlorid. If iron alone is used, it is preferred to add sufficient iron so that the resulting alloy contains about 30% of iron. The iron is preferably added periodically in about four batches. The iron becomes hot in the bath and alloys with the molten cerium, etc. The layer of barium chlorid prevents oxidation of both metals. If there is not sufficient barium chlorid in the crucible so that portions of the iron wire protrude, these portions are covered with some barium chlorid to prevent oxidation and the heating continued until they are all melted into the alloy. Before the addition of any subsequent batch of iron, the previous batch of iron should be thoroughly absorbed. During the addition of the iron, care should be taken not

to stir the batch any more than is absolutely necessary. When all the iron or other metal is added, an additional layer of barium chlorid may be added, if necessary, and the temperature raised to about 1,000° C., which increases the fluidity of the molten metal. A layer of hardened chlorid forms on the surface of the melt and keeps the rest of the batch out of contact with the air. When the melt is fairly liquid, and about ten minutes before it is poured out, it is thoroughly, but gently, stirred to produce a homogeneous mass. It is important to increase the fluidity in order that, when poured into the molds the molten metal will not be congealed prematurely as more clearly pointed out herein-after.

When the metal is thoroughly molten and homogeneous, the crucible is lifted out of the furnace and a hole poked through the crust, if any, of barium chlorid adjacent the side of the crucible, by means of a hot, thin iron bar or rod. The molten metal is then poured through this hole out into suitable molds. It is desirable to make up melts of metal of over 350 grams, preferably about 2-3 kilograms, as, if smaller melts, say of 200 grams, are used, difficulty is encountered in pouring the metal.

While any form of molds may be used, it is preferred to make them of iron. However, graphite and other materials may be used for the molds. The mold, especially if made of iron, should be uniformly heated to about 400° C. It should be over 100° C. This heating of the mold permits the pouring of the metal at a temperature so near to the solidifying point that excessive burning is avoided and at the same time permits this metal, near to the point of congelation, to find its way into and fill the mold. The mold should be slowly and uniformly heated to prevent warping thereof. By thus heating the metal mold the residual heat absorbing capacity of the mold, up to the temperature of congelation of the molten metal is reduced to a point where it does not materially affect the homogeneity of the resulting casting by causing cracks and breaks in the casting caused by rapid and uneven cooling of the molten metal. This may be accomplished, in other ways. Instead of heating a heavy metal mold a thin sheet metal mold having little heat absorbing capacity may be used to accomplish the same result as will be readily apparent to those skilled in the art. In Figs. 2, 3 and 4, there is illustrated an iron mold composed of two parts 10 and 11, the part 10 being a flat iron plate, and the part 11 being a flat iron plate, provided with grooves 12, extending from the top nearly to the bottom thereof. A connecting groove 13 is provided at the top. The plates may be held together by four angle bars 14 running along near the top and bottom on the outside of the plates 150

and pulled together by bolts 15. As clearly appears from Figs. 2 to 6 the resulting castings have relatively great length and the ratio between the volume of the casting and the area of the molding surface from which withdrawal of heat may take place is less than the ratio of 1 cubic inch of metal to 15 square inches of molding surface. In order that this relatively large heat withdrawal surface may not cause premature congealation in the mold and prevent the complete flow of molten metal into the mold, the chilling capacity of the mold is reduced as above described and the fluidity of the molten metal is increased prior to pouring by stirring and by a slight increase in the temperature thereof, as above described.

Before pouring the metal into the mold, the surfaces of the mold are dusted or otherwise coated with a layer of magnesia or other finely-divided inert material, so that the pieces of cast metal may be easily removed from the mold. The metal is poured into the connecting slot 13 and runs into the mold slots 12, filling them up. The mold should be allowed to cool slowly, that is, no artificial means are used to hasten the cooling, but the mold is allowed to air cool, and if the coating of magnesia has been uniform, a slight tapping of the plate 11, after plate 10 has been removed therefrom, should so loosen the pieces of cast metal that they may be easily removed.

In Fig. 5 is shown a top view of a similar mold adapted to form cylindrical-shaped castings or sticks of metal, and in Fig. 6 is shown a top view of a similar mold adapted to cast sticks of metal rectangular in cross-section. The resulting cast sticks of metal as they come from the molds shown in Figs. 2 to 6 are especially adapted for sparking purposes and differ materially from the pieces of alloy heretofore used for this purpose and which were made by sawing or turning under oil. The alloy castings made according to our process, have matt unsmeared glassy surfaces where formed adjacent the metal mold surfaces. While the surfaces may be somewhat rough owing to the presence of some air or blow holes on the surface, yet the surfaces have a characteristic glassy appearance and the metal is not smeared over as is the case when the pieces are formed by sawing or turning. Moreover, especially when cast in the metal molds, it is found that the castings at said surfaces have a superficial skin composed of the alloy, but poorer in the rare earth metal than is the alloy in the interior of the cast piece. This probably is due to the alloy taking up metal or particles from metal mold surface. This skin serves as a substantially non-corrosive coating or layer while having the necessary sparking properties. By melting and pouring the alloyed metals from beneath a fused salt as above described

flakes of oxid, which would otherwise be present in the casting, are substantially eliminated and the resultant casting is extremely homogeneous.

In many cases, it is found that crude metal (chiefly cerium or lanthanum), as taken from the electrolytic cell in which it is produced, is so impure or non-homogeneous that a stable and sufficiently air-resistant alloy is not produced by a single fusion of the crude metal under the purifying bath, as of barium chlorid. In such case, it is desirable to make two or more successive fusions as described, preferably before alloying (raising the melting point) and casting into final shapes (separating the metal or alloy into small pieces). After each such preliminary purifying fusion, the slag or fused salt may be removed from the crucible and fresh purifying salt already dehydrated added to the metal therein, or the metal may be cast into pigs of convenient size (about 1x1x4 inches) for remelting or for breaking into lumps for remelting.

While it has been suggested that in the making of certain brass, bronze and steel alloys, the metal may be melted below a layer of borax or waterglass, this is a very different proposition from the making of castings of the rare earth metals, such as cerium or lanthanum, and their pyrophoric alloys. Cerium is not only readily oxidized when heated, but rapidly ignites, and, furthermore, has such a great affinity for oxygen that if melted below such slags as borax or waterglass, would so rapidly combine with the oxygen therein as to cause a violent reaction. With the brass, bronze and steel alloys, there is no such problem. The making of bronze, brass and steel alloys is an art distinct and separate from the art of making pyrophoric alloys of cerium and similar rare earth metals in which the metals are so chemically active that they even unite readily with carbon to form carbid.

It has also been suggested that alloys can be prepared by melting together certain quantities of a rare earth metal and aluminum under a covering layer of sodium chlorid and potassium chlorid, but unless certain additional features or precautions are employed in the process, the results are very unsatisfactory and even then barium chlorid has distinct advantages not possessed by a mixture of sodium chlorid and potassium chlorid.

Instead of using barium chlorid as a protecting layer for the molten metal, sodium chlorid and other salts inert to the rare earth metal being used, may be used which would prevent oxidation of the metal, but barium chlorid has advantages over certain other salts because of its less volatility at the working temperature. If more volatile salts are used, there is not only a corresponding

loss of the salt, but great inconvenience to the workmen results. Furthermore, it is believed that the surface tension of fused cerium and its alloys against a molten bath 5 high in barium chlorid is far more advantageous to making homogeneous castings and protecting the surface of the metal from too rapid oxidation. Copper or magnesium may also be added to the molten metal to 10 harden the resulting alloy, or increase the fatness and heat of the spark. Other methods preventing oxidation of the melt may be used, as by carrying out the fusion in an atmosphere of hydrogen.

15 Many other changes and modifications may be made without departing from the spirit and scope of the invention in its broader aspects.

What is claimed as new and desired to be 20 secured by Letters Patent is:—

1. The process of making castings of cerium and similar rare earth metals and their alloys, which consists in melting the rare earth metal under a layer of molten 25 barium chlorid to protect the molten metal from oxidation or ignition and pouring the molten metal into molds.

2. In the process of making castings of cerium and similar rare earth metals and 30 their alloys, the steps which consist in melting the rare earth metal below a layer of a molten salt inert to the rare earth metal and protecting the molten metal from oxidation, and then introducing an alloying metal into 35 the molten rare earth metal through the layer of protecting salt.

3. In the process of making castings of cerium and similar rare earth metals and 40 their alloys, the steps which consist in melting the rare earth metal below a layer of a molten salt inert to the rare earth metal protecting the molten metal from oxidation, and introducing an alloying metal and melting the same with the rare earth metal and 45 then stirring the melt and raising the temperature of the melt to increase the fluidity thereof before pouring.

4. In the process of making castings of cerium and similar rare earth metals and 50 their alloys, the steps which consist in melting a protecting salt inert to the rare earth metal in a suitable vessel and introducing the rare earth metal in the form of pieces about one-half inch in diameter or 55 larger into the molten salt and below the surface thereof, causing the rare earth metal to melt and fall to the bottom of the bath.

5. The process of making castings of cerium and similar rare earth metals and 60 their alloys which consists in melting a protecting salt inert to molten cerium and lanthanum, in a suitable vessel and introducing the rare earth metal into the molten salt and below the surface thereof, causing

the rare earth metal to melt and fall to the 65 bottom of the bath.

6. In the process of making castings of cerium and similar rare earth metals and their alloys the steps which consist in preparing pieces of the rare earth metal, washing oxides and dirt from the surfaces thereof with volatile organic liquid, melting a layer of a protecting salt inert to the rare earth metal, and introducing the washed pieces into the molten salt and below the 75 surface thereof, causing the rare earth metal to melt and fall to the bottom of the batch.

7. In the process of making castings of alloys of cerium or lanthanum, the steps which consist in melting rare earth metal 80 containing mainly cerium or lanthanum and containing about 10% or less of iron, below a layer of molten salt inert to cerium and after the rare earth metal containing about 10% or less of iron is melted, then adding thereto an alloying metal to harden 85 the resulting alloy.

8. In the process of making castings of alloys of cerium or lanthanum, the steps which consist in melting rare earth metal 90 containing mainly cerium or lanthanum beneath a layer of molten salt inert to cerium, and adding thereto iron in the form of iron wire.

9. The process of making castings of alloys of cerium or lanthanum which consists in melting rare earth metal containing mainly cerium or lanthanum beneath a layer of molten salt inert to cerium, the resulting melt of metal being about 350 grams or over, 100 and pouring the molten metal to be cast.

10. In the process of making castings of cerium and similar rare earth metals and their alloys, the steps which consist in purifying and consolidating the metal by repeated fusion with a purifying bath of fused salt inert to the rare earth metal.

11. In the process of making castings of cerium and similar rare earth metals and their alloys, the steps which consist in purifying and consolidating the metal by repeated fusion with a purifying bath containing fused barium chlorid.

12. In the process of making castings of cerium and similar rare earth metals and 115 their alloys, the steps which consist in melting and dehydrating a salt which is inert to the rare earth metal, introducing lumps of the rare earth metal into and below the surface of the molten salt, and melting the rare 120 earth metal below said surface.

13. In the process of making castings of cerium and similar rare earth metals and their alloys, the steps which consist in melting and dehydrating a salt which is inert to 125 the rare earth metal, introducing lumps of the rare earth metal into and below the surface of the molten salt, and melting the rare

earth metal below said surface, and then introducing an alloying metal through said surface and melting the alloying metal beneath said surface to form an alloy thereof 5 with the rare earth metal.

14. In the process of making castings of cerium and similar rare earth metals, the step which consists in melting the crude metal below a layer of molten salt inert to 10 the rare earth metal to segregate impurities from the molten metal.

15. In the process of making casting of pyrophoric alloys of cerium and similar rare earth metals, the steps which consist in 15 first preparing the metal for alloying, by fusion beneath the surface of a fused salt inert to the metal and capable of segregating impurities therefrom, and then refusing the metal under a fresh batch of fused 20 salt and adding an alloying metal to the fused metal.

16. In the process of making castings of cerium and similar rare earth metals and their alloys, the steps which consist in melting 25 a salt which is inert to the molten rare earth metal or alloy thereof, melting the metal to be cast below the surface of said fused salt, pouring the molten metal into molds to form castings in which the ratio 30 between the volume of cast molten metal and the area of the molding surface from which radiation of heat may take place is

in the ratio of 1 cubic inch of metal to 15 square inches or less of molding surface, and raising the temperature of the molten metal 35 before casting to increase the fluidity of the molten metal, whereby the large heat withdrawing surface for the molten metal in the mold, will not prevent flow of molten metal into the mold by premature congealation of 40 the metal.

17. The new article of manufacture comprising a cast piece of an alloy of cerium or lanthanum, and a hardening metal, adapted for sparking purposes and having matt un- 45 smeared glassy surfaces where formed adjacent the casting mold, the casting at said surfaces having a superficial skin composed of the alloy but poorer in rare earth metal than the alloy in the interior of the cast 50 piece, said skin serving as a substantially non-corrosive coating or layer while having the necessary sparking properties, said casting being substantially free from flakes of oxid and the interior of the casting being 55 substantially homogeneous.

Signed at New York in the county of New York and State of New York this 15<sup>th</sup> day of September A. D. 1917.

ALCAN HIRSCH,  
MARX HIRSCH.

Witnesses:

JAMES N. TIMMERMANN,  
GORHAM CROSBY.